

# UNITED STATES PATENT OFFICE.

CECIL L. SAUNDERS, GEORGE C. STANLEY, AND CHARLES W. BENNETT, OF ITHACA,  
NEW YORK.

## FIREPROOF FABRIC AND PROCESS OF PRODUCING THE SAME.

1,358,250.

Specification of Letters Patent.

Patented Nov. 9, 1920.

No Drawing.

Application filed October 13, 1919. Serial No. 330,384.

*To all whom it may concern:*

Be it known that we, CECIL L. SAUNDERS, GEORGE C. STANLEY, and CHARLES W. BENNETT, all citizens of the United States,

5 residing at Ithaca, in the county of Tompkins and State of New York, have invented certain new and useful Improvements in Fireproof Fabrics and Processes of Producing the Same; and we do hereby de-  
clare the following to be a full, clear, and exact description of the invention, such as will enable others skilled in the art to which it appertains to make and use the same.

This invention relates to a composition of 15 matter, and a method of producing the same which is applicable to the fire proofing of fabrics in general, and especially the fire proofing of aeroplane wings.

The object of the invention is to provide 20 a composition and a method which is less costly, and more efficient in practice than those heretofore proposed.

With this and other objects in view the invention consists in the novel composition 25 of matter, and in the steps and combinations of steps for producing the same, all as will be more fully hereinafter disclosed and particularly pointed out in the claims.

In order that the precise invention may 30 be the more clearly understood, it is said:— It is well known that the fabrics from which aeroplane wings are produced are often subjected to fire risks, and that it is very desirable indeed to so fire proof said fabrics 35 without destroying their strength that should they become ignited, the flame will not spread and the aviator may thereupon reach a landing in safety.

It is also well known that it is very desirable to coat fabrics in general with a fire 40 proofing material, having the above mentioned characteristics, but in all of the materials and methods with which we are acquainted, various objections exist.

45 That is to say, prior processes either rot the fabrics, or the flames will spread unduly, or it is so expensive to apply the coating that they have not proved satisfactory in service. Especially has it been found in the 50 prior processes that the fire proofing coating, whatever it may be, is easily washed out, so that after the fabric has been subjected to serious wettings, its fire proofing qualities are greatly deteriorated.

55 Further, it has been found in practice that

it is a very difficult matter indeed to so open up the fibers of the material that the fire proofing substances will thoroughly penetrate the same.

In the invention, now to be described, all 60 the above objections are done away with, as will presently appear. That is to say, we have discovered that although hydrofluoric acid will readily destroy the fibers of the fabrics in general, yet, if a fabric such as 65 cotton, is first boiled in water, to remove the size, and then treated with a weak solution of hydrofluoric acid, say about two parts in one hundred parts of water, as by dipping the said fabric for thirty minutes 70 in the solution, and if it is then washed, and brought to a semi-dry state, the fabric will be found not to be weakened at all, but even strengthened to a degree.

Its pores will also be found to be so open 75 that it will readily take the fire proofing solution.

After the above mentioned treatment with hydrofluoric acid, we next may pass the fabric through a solution of sodium stannate, 80 preferably having a specific gravity of 1.075. The fabric is subjected to this last mentioned solution for about say one half minute, or somewhat longer, whereupon it is wrung out and dried. We then pass the 85 said fabric through a solution of ammonium sulfate, preferably having a specific gravity of about 1.045 and it is subjected to this last mentioned solution for about the same time as just stated, or about say one 90 minute or a little longer.

The fabric is now taken out of this ammonium sulfate solution whereupon it may be wrung out and dried, or it may be washed with water and dried. The fibers of the 95 fabric, if closely examined will be found to be coated with hydrated oxid of tin or stannic acid.

The reaction may be stated as follows:—  
$$\text{Na}_2\text{SnO}_3 \cdot x\text{H}_2\text{O} + (\text{NH}_4)_2\text{SO}_4 =$$
  
$$\text{Na}_2\text{SO}_4 + 2\text{NH}_3 + \text{SnO}_2 \cdot y\text{H}_2\text{O}$$
 100

This said hydrated oxid of tin  $\text{SnO}_2 \cdot x\text{H}_2\text{O}$  is in an exceedingly finely subdivided condition, and it functions as a most 105 efficient fire proofing material or agent for preventing the spreading of flame, whether it be applied to fabrics, to the fibers before the fabrics are made up, or even to wood. Whereas, the above treatment is found to 110

be efficient in practice, our preferred process consists in the following:—

We take a mixture of sodium stannate and of ammonium sulfate, as above mentioned, 5 but preferably in the solid condition, and grind them together until the fumes of ammonia come off, whereupon we add to the mixture any suitable varnish. This varnish may be of a gummy or resinous nature, or it 10 may be the well known varnish that is now used on aeroplane wings, which is a cellulose nitrate, or a cellulose acetate. After the varnish is thus mixed with the above reagents, the grinding is continued until we 15 have produced a thorough and intimate mixture of the varnish, and the hydrated tin oxide that is produced by the reaction during the grinding operation.

As this reaction cannot, under the circumstances, be a complete reaction, the varnish will be thus intimately mixed not only with the hydrated tin oxide, above mentioned, but there will also be present some ammonium sulfate, as well as some sodium stannate, and undoubtedly some sodium sulfate too, all of which ingredients are good fire proofing reagents. The presence of the ammonium ion undoubtedly has a good effect in causing a thorough incorporation of the 30 hydrated tin oxide into the fibers of the fabric, when the varnish containing said ingredients is applied thereto. Especially will this incorporation be very thorough if the fabric has been previously treated with the 35 hydrofluoric acid solution above mentioned.

The varnish, whether it be a resinous one or one having a cellulose base, after being thus emulsified, so to speak, with the fire proofing substances above mentioned, constitutes an article of commerce in itself, and 40 we wish it to be distinctly understood that this invention relates broadly to such a composition no matter to what substances it may be applied. Further, although this said varnish may be made by other processes, than 45 that mentioned, yet, we prefer to produce the varnish in the manner above disclosed because it is an efficient way to import into the varnish a number of fire proofing agents 50 which serve, together with the former treatment of the fibers, to so thoroughly impregnate the same that in practice the product is found to resist fire to a degree much higher

than those produced by other methods with which we are acquainted.

55

It is obvious that those skilled in the art may vary the details of the process, as well as the composition of the product without departing from the spirit of the invention, and therefore, we do not wish to be limited 60 to the above disclosure except as may be required by the claims.

What we claim is:—

1. The herein described new article of manufacture comprising a fabric having its 65 fibers coated with a fire proofing compound comprising a hydrated oxid of tin and ammonium sulfate, substantially as described.

2. The herein described new article of manufacture comprising a fabric having its 70 fibers coated with a fire proofing compound comprising a varnish having incorporated therein a hydrated oxid of tin and ammonium sulfate, substantially as described.

3. The process of rendering cotton fibers 75 more easily impregnated with sodium stannate which consists in boiling said fibers in water, treating the boiled fibers with a solution of commercial hydrofluoric acid having a strength of substantially two parts of acid 80 to 100 parts of water, washing said fibers; and bringing them to a semi-dry state, substantially as described.

4. The process of fireproofing fabrics 85 which consists in first treating said fabrics with hydrofluoric acid and then coating their fibers with a material containing a hydrated oxid of tin, substantially as described.

5. The process of fire proofing fabrics 90 which consists in first treating said fabrics with hydrofluoric acid and then coating their fibers with a material comprising a varnish, containing a hydrated oxid of tin, substantially as described.

6. The process of fire proofing fabrics 95 which consists in first treating said fabrics with hydrofluoric acid and then coating their fibers with a material comprising a varnish, containing a hydrated oxid of tin; and sodium stannate, substantially as described. 100

In testimony whereof we affix our signatures.

CECIL L. SAUNDERS.  
GEORGE C. STANLEY.  
CHARLES W. BENNETT.